# EUROPEAN PATENT SPECIFICATION

(11) **EP 2 837 700 B1**
(45) Date of publication and mention of the grant of the patent: **05.06.2019**
(21) Application number: 13776255.5
(22) Date of filing: 05.04.2013
(51) Int. Cl.: C21D 9/56, C21D 1/74, C21D 1/76, F27D 7/04, F27D 17/00, F27D 7/06, C21D 9/52

(54) **METHOD FOR LOWERING DEW POINT OF ATMOSPHERE GAS WITHIN ANNEALING FURNACE, DEVICE THEREOF, AND METHOD FOR PRODUCING COLD-ROLLED ANNEALED STEEL SHEET**
VERFAHREN ZUM SENKEN DES TAUPUNKTES VON UMGEBUNGSGAS IN EINEM GLÜHOFEN, VORRICHTUNG DAFÜR UND VERFAHREN ZUR HERSTELLUNG VON KALTGEWALZTEM GEGLÜHTEM STAHLBLECH
PROCÉDÉ POUR RÉDUIRE LE POINT DE ROSÉE DE GAZ AMBIANT DANS UN FOUR DE RECUIT, DISPOSITIF ASSOCIÉ, ET PROCÉDÉ DE PRODUCTION DE TÔLE D'ACIER RECUIT LAMINÉE À FROID

(30) Priority: 09.04.2012 JP 2012088089
(43) Date of publication of application: 18.02.2015
(73) Proprietor: JFE Steel Corporation, Tokyo, 100-0011 (JP)
(72) Inventor: FUJII, Takamasa, Tokyo 100-0011 (JP); IRI, Masato, Tokyo 100-0011 (JP)
(74) Representative: Grünecker Patent- und Rechtsanwälte PartG mbB
(86) International application number: PCT/JP2013/002353
(87) International publication number: WO 2013/153791

(56) References cited:
- EP-A2- 0 976 842
- WO-A1-2012/081719
- GB-A- 1 297 410
- JP-A- H0 347 923
- JP-A- H02 236 229
- JP-A- H10 176 225
- JP-A- H11 124 622
- JP-A- 2000 104 123

## Description

### Technical Field

The present invention belongs to the field of advantageous production of a steel strip that can reduce the dew point of an atmosphere gas in a continuous annealing furnace and has high wettability and, in particular, relates to a method for reducing the dew point of an atmosphere gas in an annealing furnace, an apparatus for the method, and a method for producing a cold-rolled and annealed steel sheet.

### Background Art

It is known that when the dew point of an atmosphere gas in a continuous annealing furnace is -45°C or less, surface segregation of Mn during annealing can be suppressed, and the adhesion of zinc or zinc alloy plating after annealing is improved (see Non Patent Literature 1).

The following are examples of a method in the related art for reducing the dew point of an atmosphere gas in a continuous annealing furnace.
A: A method for supplying another atmosphere gas having a low dew point from the outside of a furnace to a heating zone or a soaking zone (see Patent Literature 1).
B: A method for providing a mechanism for circulating a furnace atmosphere gas in the outside of the furnace and thereby performing heat exchange between the circulating high-temperature atmosphere gas and a room-temperature atmosphere gas having a low dew point, which is to be supplied separately to the furnace (see Patent Literature 2).
C: A method for performing heat exchange between a high-temperature furnace atmosphere gas and an atmosphere gas having a dew point that has been reduced in the outside of a furnace and reducing the dew point with a water adsorption filter (see Patent Literature 3).

### Citation List

### Patent Literature

PTL 1: Japanese Unexamined Patent Application Publication No. 2002-3953
PTL 2: Japanese Unexamined Patent Application Publication No. 62-290830
PTL 3: Japanese Unexamined Patent Application Publication No. 11-124622

### Non Patent Literature

NPL 1: Tetsu To Hagane (Bulletin of the Iron and Steel Institute of Japan), 96-1 (2010), pp. 11-20

### Summary of Invention

### Technical Problem

In accordance with the related art A, the low-temperature gas is directly introduced into the high-temperature furnace. Thus, a large amount of thermal energy is required to maintain the steel strip temperature in the furnace, the gas temperature cannot be controlled, and the energy efficiency is very low.

In accordance with the related art B, even when the low-temperature gas has a low dew point, the low-temperature gas is mixed with a large amount of atmosphere gas having a high dew point in the furnace. Thus, the dew point of the atmosphere gas in the furnace cannot be sufficiently reduced.

In accordance with the related art C, the temperature of a gas to be returned to the furnace is not sufficiently increased and, as described in Patent Literature 3, the water adsorption filter having a low dehumidification capacity reduces the dew point only to approximately -30°C and cannot reduce the dew point to -45°C or less, which is a target of the present application. Thus, known techniques for reducing the dew point of the atmosphere of a continuous annealing furnace have problems that they cannot achieve a low dew point of -45°C or less and that they have very low energy efficiency.

### Solution to Problem

As a result of extensive studies to solve the problems described above, the present inventors completed the present invention by considering means for installing a dryer, for example, of a desiccant method or a compressor method that allows a dew point of -45°C or less in order to reduce the dew point of an annealing furnace atmosphere gas and a circulator to reduce the dew point to -45°C, installing a heat exchanger in the circulator to increase or decrease the temperature of the gas, and modifying a gas inflow (gas introduction) into a heating zone and a cooling zone of the furnace to improve energy efficiency.

The present invention can be summarized as follows:
(1) A method for reducing the dew point of a furnace atmosphere gas in a continuous annealing furnace for annealing a metal strip in a reducing atmosphere by passing the metal strip through a heating zone and a cooling zone in this order or through a heating zone, a soaking zone, and a cooling zone in this order, including:
   a step (a) for providing a circulator that includes a heat exchanger for heat exchange between a low-temperature gas and a high-temperature gas, a gas cooler for cooling a gas, and a dryer for dehumidifying a gas to a dew point of - 45°C or less;
   a step (b) for sucking part of the atmosphere gas from the heating zone and/or the soaking zone;
   then a step (c) for passing the sucked part of the atmosphere gas through a high-temperature gas passage of the heat exchanger and decreasing the temperature of the sucked part of the atmosphere gas by heat exchange with a gas in a low-temperature gas passage;
   then a step (d) for mixing the part of the atmosphere gas having a decreased temperature with part of an atmosphere gas sucked from the cooling zone to further decrease the temperature of the part of the atmosphere gas;
   then a step (e) for passing the part of the atmosphere gas further cooled by mixing with the part of the atmosphere gas sucked from the cooling zone through the gas cooler to further cooling the part of the atmosphere gas;
   then a step (f) for dehumidifying the part of the atmosphere gas further cooled through the gas cooler to a dew point of -45°C or less in the dryer;
   then a step (g) for passing the dehumidified part of the atmosphere gas through the low-temperature gas passage of the heat exchanger to increase the temperature of the dehumidified part of the atmosphere gas by heat exchange with a gas in the high-temperature gas passage; and
   then a step (h) for returning the part of the atmosphere gas having an increased temperature to the heating zone and/or the soaking zone.
(2) The method for reducing the dew point of an atmosphere gas in an annealing furnace according to (1), wherein the part of gas flowing from the dryer toward the low-temperature gas passage of the heat exchanger is returned directly to the cooling zone without passing through the heat exchanger.
(3) An apparatus for reducing the dew point of an atmosphere gas in a continuous annealing furnace for annealing a metal strip in a reducing atmosphere by passing the metal strip through a heating zone 1 and a cooling zone 2 in this order or through a heating zone, a soaking zone, and a cooling zone in this order, comprising:
   a gas passage including a heat exchanger 9 for heat exchange between a low-temperature gas and a high-temperature gas, a gas cooler 10 for cooling a gas, a dryer 11 for dehumidifying a gas to a dew point of -45°C or less, and a gas mixer 20,
   wherein the apparatus includes
   a gas passage extending from the heating zone 1 and/or the soaking zone through a gas passage 15 to a high-temperature gas passage of the heat exchanger 9 and through the gas cooler 10 to the dryer 11,
   a gas passage 16 extending from the dryer 11 to a low-temperature gas passage of the heat exchanger 9 and from the heat exchanger 9 to the heating zone and/or the soaking zone, and
   a gas passage 19 extending from the cooling zone 2, the gas passage 19 being connected to a gas passage extending from the heat exchanger 9 to the gas cooler 10 in the gas mixer 20.
(4) The apparatus for reducing the dew point of an atmosphere gas in an annealing furnace according to (3), further comprising a gas passage 17 for returning part of gas flowing from the dryer 11 toward the low-temperature gas passage of the heat exchanger 9 directly to the cooling zone through a gas distributor 13 but without passing through the heat exchanger 9.
(5) A method for producing a cold-rolled and annealed steel sheet, comprising continuously annealing a cold-rolled steel strip, wherein
   the dew point of an atmosphere gas in the continuous annealing furnace according to (1) or (2) is reduced by the method for reducing the dew point of an atmosphere gas in an annealing furnace according to (1) or (2) during the continuous annealing.

### Advantageous Effects of Invention

In accordance with the present invention, part of an atmosphere gas in the heating zone and/or the soaking zone is sucked out and is cooled through a high-temperature gas passage of the heat exchanger by heat exchange with a gas in a low-temperature gas passage, is then further cooled by mixing with part of an atmosphere gas of the cooling zone, is then further cooled through the gas cooler, is then dehumidified to a dew point of -45°C or less in the dryer, is then heated through the low-temperature gas passage of the heat exchanger by heat exchange with a gas in the high-temperature gas passage, and is returned to the heating zone and/or the soaking zone. More preferably, part of gas flowing from the dryer toward the low-temperature gas passage of the heat exchanger is returned directly to the cooling zone without passing through the heat exchanger. These can achieve a very low dew point of -45°C or less in the annealing furnace and significantly improve energy efficiency.

### Brief Description of Drawings

Fig. 1 is a schematic view of Conventional Example 1.
Fig. 2 is a schematic view of Conventional Example 2.
Fig. 3 is a schematic view of a circulation system according to Conventional Example 2.
Fig. 4 is a schematic view of Conventional Example 3.
Fig. 5 is a schematic view of a circulation system according to Conventional Example 3.
Fig. 6 is a schematic view of Comparative Example 1.
Fig. 7 is a schematic view of a circulation system according to Comparative Example 1.
Fig. 8 is a schematic view of Example 1 of the present invention.
Fig. 9 is a schematic view of a circulation system according to Example 1 of the present invention.
Fig. 10 is a schematic view of Example 2 of the present invention.
Fig. 11 is a schematic view of a circulation system according to Example 2 of the present invention. Description of Embodiments

When a cold-rolled steel strip is continuously annealed and is subsequently plated with zinc or a zinc alloy, the adhesion of plating depends greatly on the dew point in an annealing furnace. It is known that this results from the amount of Mn oxide on the surface of the steel strip. At a dew point in the vicinity of -10°C, Mn oxide is present within an oxide film on the surface of the steel strip and is rarely found on the surface of the steel strip. At a dew point of -45°C or less, Mn oxide is negligibly produced. At an intermediate dew point in the vicinity of -35°C (-15°C to -40°C), a large amount of Mn oxide is produced on the surface of the steel strip and inhibits the adhesion of plating. Thus, the present inventors considered providing the annealing furnace with a circulator equipped with a dryer that allows a dew point of -45°C or less in order to achieve a very low dew point to prevent concentration of Mn oxide on the surface of the steel strip.

Attention is now focused on the temperatures of an atmosphere gas sucked from the furnace into the circulator (hereinafter referred to as a sucked gas) and an atmosphere gas introduced from the circulator into the furnace (hereinafter referred to as an introduced gas). The desired atmosphere gas temperature in the annealing furnace is different in a heating zone, a soaking zone, and a cooling zone. More specifically, the sucked gas is cooled to approximately room temperature in a gas cooler before entering the dryer, is dehumidified in the dryer, and is returned to the furnace. Thus, if a low-temperature gas is directly introduced into a high-temperature region, such as the heating zone or the soaking zone, a high temperature required for annealing the steel strip cannot be maintained. For this reason, the temperature of the introduced gas from the circulator must be increased.

The present inventors employed a method for installing a heat exchanger between the furnace and the gas cooler. More specifically, a high-temperature gas sucked from the heating zone or the soaking zone of the furnace (sucked gas) is cooled in the cooler before entering the dryer. Utilizing thermal energy resulting from the temperature difference, therefore, the gas cooled in the gas cooler and dehumidified in the dryer can be heated. Thus, thermal energy discharged from the gas cooler can be effectively utilized. A high-temperature gas sucked from the heating zone or the soaking zone of the furnace is passed through the heat exchanger, is cooled in the gas cooler, is dehumidified in the dryer, is heated in the heat exchanger, and is then returned to the heating zone or the soaking zone of the furnace.

The temperature of the high-temperature gas sucked from the heating zone or the soaking zone after the heat exchange is sometimes higher than the gas temperature in the cooling zone. Thus, the gas after the heat exchange can advantageously be mixed with a low-temperature gas sucked from the cooling zone to reduce energy required to further cool the gas in the downstream gas cooler.

Furthermore, since the gas temperature after cooling with the gas cooler is lower than the temperature of the cooling zone of the furnace, part of gas cooled in the gas cooler, dehumidified in the dryer, and returned directly to the cooling zone without passing through the heat exchanger can reduce the temperature and the dew point of the cooling zone, thus further improving energy efficiency.

Unlike a water adsorption filter made of activated alumina, alternately operated and stopped, and having a low dehumidification capacity as described in Patent Literature 3, a dryer for use in the present invention preferably has a high dehumidification capacity, for example, of a desiccant method for continuous dehumidification using calcium oxide, zeolite, silica gel, or calcium chloride or a compressor method using an alternative chlorofluorocarbon.

### EXAMPLES

Figs. 1 to 11 illustrate the structure and gas passages of a continuous annealing furnace having a heating zone and a cooling zone according to Examples, Comparative Example, and Conventional Examples.

Fig. 1 illustrates Conventional Example 1 described in Patent Literature 1. Atmosphere gas supply equipment 12 directly supplies another low-temperature atmosphere gas to a heating zone 1 and a cooling zone 2.

Figs. 2 and 3 illustrate Conventional Example 2 described in Patent Literature 2. A gas sucked from a cooling zone 2 enters a circulator 8 through a flow path 15, passes through a heat exchanger 9 to heat a gas from atmosphere gas supply equipment 12, and returns to the cooling zone 2 through a flow path 16. The low-temperature atmosphere gas supplied from the gas supply equipment 12 is heated in the heat exchanger 9 and is introduced into a heating zone 1 through an atmosphere gas pipe 7.

Figs. 4 and 5 illustrate Conventional Example 3 described in Patent Literature 3. A gas sucked from heating zone 1 is introduced into a circulator 8 through a flow path 15, is cooled in a heat exchanger 9 with a gas from a water adsorption filter 18, is dehumidified with the water adsorption filter 18 made of activated alumina, is heated in the heat exchanger 9, and is returned to the heating zone 1 through a flow path 16. Each apparatus includes three water adsorption filters 18, which are alternately operated at intervals of three hours.

Figs. 6 and 7 illustrate Comparative Example 1. A gas sucked from a heating zone 1 is introduced into a circulator 8 through a flow path 15, is cooled in a heat exchanger 9 with a gas that has been dehumidified in a dryer 11, is further cooled in a gas cooler 10, is dehumidified in the dryer 11, is heated in the heat exchanger 9 with a gas from the heating zone 1, and is returned to the heating zone 1 through a flow path 16.

Figs. 8 and 9 illustrate Example 1 of the present invention and correspond to (1) and (3) in Solution to Problem. A gas sucked from a heating zone 1 is introduced into a circulator 8 through a flow path 15, is cooled in a heat exchanger 9 with a dehumidified gas from a dryer, is mixed in a mixer 20 with another gas sucked from a cooling zone 2 through a flow path 19, is further cooled in a cooler 10, is dehumidified in a dryer 11, is heated with a gas from the heating zone 1, and is returned to the heating zone 1 through a flow path 16.

Figs. 10 and 11 illustrate Example 2 of the present invention and correspond to (2) and (4) in Solution to Problem. In addition to Example 1 of the present invention illustrated in Figs. 8 and 9, the gas dehumidified in the dryer 11 is distributed with a gas distributor 13. One part of the distributed gas is introduced into the heat exchanger 9, is heated therein with a gas from the heating zone 1 and is returned to the heating zone 1 through a flow path 16. The other part of the distributed gas is returned directly to a cooling zone 2 through a flow path 17.

The conditions of these sucked gases and introduced gases were changed. Table 1 shows the dew points of the sucked gases and the dew points of the introduced gases passing through the gas passages and exhausted heat energy during the passage in Examples and Conventional Examples. Table 1 shows that the dew points of the gases introduced into the annealing furnaces in No. 1 to No. 3 of Example 1 and No. 4 to No. 6 of Example 2 are satisfactorily lower than the target temperature of -45°C, as compared with Conventional Examples No. 7 to No. 10. Furthermore, the dew points in the furnaces measured upstream from an annealing furnace outlet 21 are also satisfactorily lower than -45°C. Furthermore, No. 1 to No. 3 of Example 1 and No. 4 to No. 6 of Example 2 exhausted less heat energy and have very high energy efficiency.

The adhesion of zinc alloy plating was examined in zinc alloy plating of a steel strip after continuous annealing in accordance with a JIS-H8504(g) tape test method (a chipping test method). As a result, Examples No. 1 to No. 6 had satisfactorily strong adhesion, but Conventional Examples No. 7 to No. 10 had coating defects.

**[Table 1]**

| No. | Sucked gas | | | | Introduced gas | | | | Dew point in furnace measured upstream from continuous annealing furnace outlet (°C) | Exhausted heat energy kJ/Nm³ | Dehumidification method | Adhesion of Zn alloy plating after continuous annealing | Note |
|---|---|---|---|---|---|---|---|---|---|---|---|---|---|
| | Position | Flow rate Nm³/Hr | Temperature °C | Dew point °C | Position | Flow rate Nm³/Hr | Temperature °C | Dew point °C | | | | | |
| 1 | Heating zone | 500 | 800 | -20 | Heating zone | 750 | 600 | -52 | -50 | 68 | Calcium oxide | Strong | Example 1 |
| | Cooling zone | 250 | 50 | -25 | | | | | | | | | |
| 2 | Heating zone | 500 | 850 | -25 | Heating zone | 1000 | 500 | -55 | -52 | 80 | Zeolite | Strong | Example 1 |
| | Cooling zone | 500 | 150 | -15 | | | | | | | | | |
| 3 | Heating zone | 1500 | 950 | -25 | Heating zone | 2000 | 700 | -60 | -55 | 78 | Silica gel | Strong | Example 1 |
| | Cooling zone | 500 | 20 | -15 | | | | | | | | | |
| 4 | Heating zone | 1000 | 700 | -10 | Heating zone | 1000 | 550 | -50 | -48 | 42 | Zeolite | Strong | Example 2 |
| | Cooling zone | 1000 | 200 | -10 | Cooling zone | 1000 | 20 | | | | | | |
| 5 | Heating zone | 500 | 850 | -25 | Heating zone | 250 | 600 | -51 | -49 | 35 | Calcium chloride | Strong | Example 2 |
| | Cooling zone | 1500 | 30 | -15 | Cooling zone | 1750 | 25 | | | | | | |
| 6 | Heating zone | 2000 | 950 | -15 | Heating zone | 1500 | 600 | -70 | -65 | 40 | Compressor method | Strong | Example 2 |
| | Cooling zone | 500 | 20 | -25 | Cooling zone | 1000 | 5 | | | | | | |
| 7 | Cooling zone | 0 | - | - | Cooling zone | 3000 | 25 | -50 | -35 | 253 | - | Coating defect | Conventional example 1 |
| 8 | Heating zone | 0 | - | - | Heating zone | 1500 | 5 | -45 | -32 | 402 | - | Coating defect | Conventional example 1 |
| 9 | Heating zone | 500 | 950 | -20 | Heating zone | 500 | 700 | -20 | -21 | 155 | - | Coating defect | Conventional example 2 |
| | | | | | | (250) | 200 | -40 | | | | | |
| 10 | Heating zone | 4000 | 800 | -15 | Heating zone | 4000 | 600 | -35 | -23 | 189 | - | Coating defect | Conventional example 2 |

| | | | | | | | | | | | | | |
|---|---|---|---|---|---|---|---|---|---|---|---|---|---|
| [Note] A flow rate in parentheses is the flow rate of another supplied gas. | | | | | | | | | | | | | |

### Reference Signs List

1 Heating zone
2 Cooling zone
3 Steel strip
4 Roller
5 Suction port
6 Inlet
7 Atmosphere gas pipe
8 Circulator
9 Heat exchanger
10 Gas cooler
11 Dryer (dehumidifier)
12 Equipment for supplying another atmosphere gas
13 Gas distributor
15 Gas flow path from heating zone
16 Gas flow path to heating zone
17 Gas flow path to cooling zone
18 Water adsorption filter
19 Gas flow path from cooling zone
20 Gas mixer
21 Annealing furnace outlet

## Claims

1. A method for reducing the dew point of a furnace atmosphere gas in a continuous annealing furnace for annealing a metal strip in a reducing atmosphere by passing the metal strip through a heating zone and a cooling zone in this order or through a heating zone, a soaking zone, and a cooling zone in this order, comprising:
a step (a) for providing a circulator that includes a heat exchanger for heat exchange between a low-temperature gas and a high-temperature gas, a gas cooler for cooling a gas, and a dryer for dehumidifying a gas to a dew point of - 45°C or less;
a step (b) for sucking part of the atmosphere gas from the heating zone and/or the soaking zone;
then a step (c) for passing the sucked part of the atmosphere gas through a high-temperature gas passage of the heat exchanger and decreasing the temperature of the sucked part of the atmosphere gas by heat exchange with a gas in a low-temperature gas passage;
then a step (d) for mixing the part of the atmosphere gas having a decreased temperature with part of an atmosphere gas sucked from the cooling zone to further decrease the temperature of the part of the atmosphere gas;
then a step (e) for passing the part of the atmosphere gas further cooled by mixing with the part of the atmosphere gas sucked from the cooling zone through the gas cooler to further cooling the part of the atmosphere gas;
then a step (f) for dehumidifying the part of the atmosphere gas further cooled through the gas cooler to a dew point of -45°C or less in the dryer;
then a step (g) for passing the dehumidified part of the atmosphere gas through the low-temperature gas passage of the heat exchanger to increase the temperature of the dehumidified part of the atmosphere gas by heat exchange with a gas in the high-temperature gas passage; and
then a step (h) for returning the part of the atmosphere gas having an increased temperature to the heating zone and/or the soaking zone.

2. The method for reducing the dew point of an atmosphere gas in an annealing furnace according to Claim 1, wherein the part of gas flowing from the dryer toward the low-temperature gas passage of the heat exchanger is returned directly to the cooling zone without passing through the heat exchanger.

3. An apparatus for reducing the dew point of an atmosphere gas in a continuous annealing furnace for annealing a metal strip in a reducing atmosphere by passing the metal strip through a heating zone 1 and a cooling zone 2 in this order or through a heating zone, a soaking zone, and a cooling zone in this order, comprising:
a gas passage including a heat exchanger 9 for heat exchange between a low-temperature gas and a high-temperature gas, a gas cooler 10 for cooling a gas, a dryer 11 for dehumidifying a gas to a dew point of -45°C or less, and a gas mixer 20,
wherein the apparatus includes
a gas passage extending from the heating zone 1 and/or the soaking zone through a gas passage 15 to a high-temperature gas passage of the heat exchanger 9 and through the gas cooler 10 to the dryer 11,
a gas passage 16 extending from the dryer 11 to a low-temperature gas passage of the heat exchanger 9 and from the heat exchanger 9 to the heating zone and/or the soaking zone, and
a gas passage 19 extending from the cooling zone 2, the gas passage 19 being connected to a gas passage extending from the heat exchanger 9 to the gas cooler 10 in the gas mixer 20.

4. The apparatus for reducing the dew point of an atmosphere gas in an annealing furnace according to Claim 3, further comprising a gas passage 17 for returning part of gas flowing from the dryer 11 toward the low-temperature gas passage of the heat exchanger 9 directly to the cooling zone through a gas distributor 13 but without passing through the heat exchanger 9.

5. A method for producing a cold-rolled and annealed steel sheet, comprising continuously annealing a cold-rolled steel strip, wherein
the dew point of an atmosphere gas in a continuous annealing furnace is reduced by the method for reducing the dew point of an atmosphere gas in an annealing furnace according to Claim 1 or 2 during the continuous annealing.

## Patentansprüche

1. Verfahren zum Reduzieren des Taupunktes eines Ofenatmosphären-Gases in einem Durchlaufglühofen, in dem ein Metallband in einer reduzierenden Atmosphäre geglüht wird, indem das Metallband durch eine Erhitzungs-Zone und eine Abkühlungs-Zone in dieser Reihenfolge oder durch eine Erhitzungs-Zone, eine Halte-Zone und eine Abkühlungs-Zone in dieser Reihenfolge geleitet wird, wobei das Verfahren umfasst:
einen Schritt (a), in dem eine Zirkulations-Einrichtung bereitgestellt wird, die einen Wärmetauscher für Wärmeaustausch zwischen einem Niedrigtemperatur-Gas und einem Hochtemperatur-Gas, einen Gas-Kühler zum Kühlen eines Gases sowie einen Trockner zum Entfeuchten eines Gases auf einen Taupunkt von - 45 °C oder darunter enthält;
einen Schritt (b), in dem ein Teil des Atmosphären-Gases aus der Erhitzungs-Zone und/oder der Halte-Zone abgesaugt wird;
danach einen Schritt (c), in dem der abgesaugte Teil des Atmosphären-Gases durch einen Hochtemperatur-Gaskanal des Wärmetauschers geleitet wird und die Temperatur des abgesaugten Teils des Atmosphären-Gases durch Wärmeaustausch mit einem Gas in einem Niedrigtemperatur-Gaskanal verringert wird;
danach einen Schritt (d), in dem der Teil des Atmosphären-Gases, der verringerte Temperatur aufweist, mit einem Teil eines aus der Abkühlungs-Zone abgesaugten Atmosphären-Gases vermischt wird, um die Temperatur des Teils des Atmosphären-Gases weiter zu verringern;
danach einen Schritt (e), in dem der Teil des durch Mischen mit dem Teil des aus der Abkühlungs-Zone abgesaugten Atmosphären-Gases weiter abgekühlten Atmosphären-Gases durch den Gas-Kühler geleitet wird, um den Teil des Atmosphären-Gases weiter abzukühlen;
danach einen Schritt (f) zum Entfeuchten des durch den Gas-Kühler weiter abgekühlten Teils des Atmosphären-Gases auf einen Taupunkt von - 45 °C oder darunter in dem Trockner;
danach einen Schritt (g), in dem der entfeuchtete Teil des Atmosphären-Gases durch den Niedrigtemperatur-Gaskanal des Wärmetauschers geleitet wird, um die Temperatur des entfeuchteten Teils des Atmosphären-Gases durch Wärmeaustausch mit einem Gas in einem Hochtemperatur-Gaskanal zu erhöhen; sowie
danach einen Schritt (h), in dem der Teil des Atmosphären-Gases, der erhöhte Temperatur aufweist, zu der Erhitzungs-Zone und/oder der Halte-Zone zurückgeführt wird.

2. Verfahren zum Reduzieren des Taupunktes eines Atmosphären-Gases in einem Glühofen nach Anspruch 1, wobei der Teil des Gases, der von dem Trockner in Richtung des Niedrigtemperatur-Gaskanals des Wärmetauschers strömt, direkt zu der Abkühlungs-Zone zurückgeführt wird, ohne durch den Wärmetauscher zu strömen.

3. Vorrichtung zum Reduzieren des Taupunktes eines Atmosphären-Gases in einem Durchlaufglühofen, in dem ein Metallband in einer reduzierenden Atmosphäre geglüht wird, indem das Metallband durch eine Erhitzungs-Zone (1) und eine Abkühlungs-Zone (2) in dieser Reihenfolge oder durch eine Erhitzungs-Zone, eine Halte-Zone und eine Abkühlungs-Zone in dieser Reihenfolge geleitet wird, wobei die Vorrichtung umfasst:
einen Gaskanal, der einen Wärmetauscher (9) für Wärmeaustausch zwischen einem Niedrigtemperatur-Gas und einem Hochtemperatur-Gas, einen Gas-Kühler (10) zum Kühlen eines Gases, einen Trockner (11) zum Entfeuchten eines Gases auf einen Taupunkt von - 45 °C oder darunter sowie einen Gas-Mischer (20) enthält;
wobei die Vorrichtung einschließt:
einen Gaskanal, der von der Erhitzungs-Zone (1) und/oder der Halte-Zone über einen Gaskanal (15) zu einem Hochtemperatur-Gaskanal des Wärmetauschers (9) sowie über den Gas-Kühler (10) zu dem Trockner (11) verläuft,
einen Gaskanal (16), der von dem Trockner (11) zu einem Niedrigtemperatur-Gaskanal des Wärmetauschers (9) und von dem Wärmetauscher (9) zu der Erhitzungs-Zone und/oder der Halte-Zone verläuft, sowie
einen Gaskanal (19), der von der Abkühlungs-Zone (2)aus verläuft, wobei der Gaskanal (19) mit einem Gaskanal, der von dem Wärmetauscher (9) zu dem Gas-Kühler (10) verläuft, in dem Gas-Mischer (20) verbunden ist.

4. Vorrichtung zum Reduzieren des Taupunktes eines Atmosphären-Gases in einem Glühofen nach Anspruch 3, die des Weiteren einen Gaskanal (17) umfasst, mit dem ein Teil des Gases, das von dem Trockner (11) in Richtung des Niedrigtemperatur-Gaskanals des Wärmetauschers (9) strömt, über einen Gas-Verteiler (13) direkt zu der Abkühlungs-Zone zurückgeführt wird, ohne durch den Wärmetauscher zu strömen (9).

5. Verfahren zum Herstellen eines kaltgewalzten und geglühten Stahlblechs, das Durchlaufglühen eines kaltgewalzten Stahlbandes umfasst, wobei
der Taupunkt eines Atmosphären-Gases in einem Durchlaufglühofen mit dem Verfahren zum Reduzieren des Taupunktes eines Atmosphären-Gases in einem Glühofen nach Anspruch 1 oder 2 während des Durchlaufglühens reduziert wird.

## Revendications

1. Procédé pour abaisser le point de rosée d'un gaz ambiant de four dans un four de recuit continu destiné à recuire une bande métallique dans une atmosphère réductrice par passage de la bande métallique à travers une zone de chauffage et une zone de refroidissement, dans cet ordre, ou à travers une zone de chauffage, une zone de maintien et une zone de refroidissement, dans cet ordre, comprenant :
une étape (a) consistant à fournir un circulateur qui inclut un échangeur de chaleur destiné à un échange de chaleur entre un gaz à basse température et un gaz à haute température, un refroidisseur de gaz destiné à refroidir un gaz et un sécheur destiné à déshumidifier un gaz jusqu'à un point de rosée de -45 °C ou moins ;
une étape (b) consistant à aspirer une partie du gaz ambiant depuis la zone de chauffage et/ou la zone de maintien ;
puis une étape (c) consistant à faire passer la partie aspirée du gaz ambiant à travers un passage de gaz à haute température de l'échangeur de chaleur et réduire la température de la partie aspirée du gaz ambiant par échange de chaleur avec un gaz dans un passage de gaz à basse température ;
puis une étape (d) consistant à mélanger la partie du gaz ambiant ayant une température réduite avec une partie d'un gaz ambiant aspiré depuis la zone de refroidissement pour réduire encore une température de la partie du gaz ambiant ;
puis une étape (e) consistant à faire passer la partie du gaz ambiant encore refroidie par mélange avec la partie du gaz ambiant aspirée depuis la zone de refroidissement à travers le refroidisseur de gaz pour refroidir encore la partie du gaz ambiant ;
puis une étape (f) consistant à déshumidifier la partie du gaz ambiant encore refroidie à travers le refroidisseur de gaz jusqu'à un point de rosée de -45 °C ou moins dans le sécheur ;
puis une étape (g) consistant à faire passer la partie du gaz ambiant déshumidifiée à travers le passage de gaz à basse température de l'échangeur de chaleur pour augmenter la température de la partie du gaz ambiant déshumidifiée par échange de chaleur avec un gaz dans le passage de gaz à haute température ; et
puis une étape (h) consistant à renvoyer la partie du gaz ambiant ayant une température augmentée dans la zone de chauffage et/ou la zone de maintien.

2. Procédé pour abaisser le point de rosée d'un gaz ambiant dans un four de recuit selon la revendication 1, dans lequel la partie de gaz s'écoulant du sécheur en direction du passage de gaz à basse température de l'échangeur de chaleur est renvoyée directement à la zone de refroidissement sans traverser l'échangeur de chaleur.

3. Appareil pour abaisser le point de rosée d'un gaz ambiant dans un four de recuit continu destiné à recuire une bande métallique dans une atmosphère réductrice par passage de la bande métallique à travers une zone de chauffage 1 et une zone de refroidissement 2, dans cet ordre, ou à travers une zone de chauffage, une zone de maintien et une zone de refroidissement, dans cet ordre, comprenant :
un passage de gaz incluant un échangeur de chaleur 9 destiné à un échange de chaleur entre un gaz à basse température et un gaz à haute température, un refroidisseur de gaz 10 destiné à refroidir un gaz, un sécheur 11 destiné à déshumidifier un gaz jusqu'à un point de rosée de -45 °C ou moins et un mélangeur de gaz 20,
l'appareil incluant
un passage de gaz s'étendant depuis la zone de chauffage 1 et/ou la zone de maintien à travers un passage de gaz 15 jusqu'à un passage de gaz à haute température de l'échangeur de chaleur 9 et à travers le refroidisseur de gaz 10 jusqu'au sécheur 11,
un passage de gaz 16 s'étendant depuis le sécheur 11 jusqu'à un passage de gaz à basse température de l'échangeur de chaleur 9 et depuis l'échangeur de chaleur 9 jusqu'à la zone de chauffage et/ou la zone de maintien, et
un passage de gaz 19 s'étendant depuis la zone de refroidissement 2, le passage de gaz 19 étant connecté à un passage de gaz s'étendant depuis l'échangeur de chaleur 9 jusqu'au refroidisseur de gaz 10 dans le mélangeur de gaz 20.

4. Appareil pour abaisser le point de rosée d'un gaz ambiant dans un four de recuit selon la revendication 3, comprenant, en outre, un passage de gaz 17 destiné à renvoyer une partie du gaz s'écoulant du sécheur 11 vers le passage de gaz à basse température de l'échangeur de chaleur 9 directement à la zone de refroidissement à travers un distributeur de gaz 13 mais sans traverser l'échangeur de chaleur 9.

5. Procédé de production d'une tôle d'acier laminée à froid et recuite, comprenant le recuit continu d'une bande d'acier laminée à froid, dans lequel
le point de rosée d'un gaz ambiant dans un four de recuit continu est abaissé par le procédé destiné à abaisser le point de rosée d'un gaz ambiant dans un four de recuit selon la revendication 1 ou 2 pendant le recuit continu.
